

Patented July 28, 1953

2,647,069

## UNITED STATES PATENT OFFICE

2,647,069

## MANUFACTURE OF SILICATE-COATED PAPERS

William Stericker, Drexel Hill, Pa., assignor to  
 Philadelphia Quartz Company, Philadelphia,  
 Pa., a corporation of Pennsylvania

No Drawing. Application January 23, 1947,  
 Serial No. 723,885

2. Claims. (Cl. 117—152)

1

This invention relates to improvements in the manufacture of silicate-coated papers; and it comprises a process of coating paper wherein a paper board or sheet, containing ligneous or other components normally subject to staining by the action of alkali, is coated with a silicate solution having a gravity within the range of about 10° to 55° Bé. and containing a small amount of a bleaching agent and an alkali metal silicate having a weight ratio of alkali metal oxide to  $\text{SiO}_2$  within the range of from about 1:1.6 to 1:4, the higher gravities being usually employed with the higher ratios of alkali metal oxide to  $\text{SiO}_2$ , the bleaching agent being advantageously present in amount sufficient to produce a bleaching action substantially equivalent to that produced by from about 0.25 to 5.0 per cent of hydrogen peroxide, whereby the discoloration of the coated paper normally caused by the alkaline silicate solution will be decreased and the paper will have a brightness which is higher than that of the sheet or board coated with alkaline silicate alone and which may be higher than that of the uncoated sheet. The invention also includes the coated paper sheet or board produced by the described process, said sheet or board being superficially bleached so that the discoloration normally caused by the alkaline sodium silicate is decreased or eliminated, the dried reaction products of the bleaching action being present in said sheet or board; all as more fully hereinafter set forth and as claimed.

There has long been an important demand in the art for papers and paper boards which are resistant to oils and greases. Such papers are useful in lining or making cookie containers, cake boxes, salve boxes, dentifrice containers, coffee bags, fiber cans, spice and cosmetic containers and the like. Papers of this type are also useful for wrapping rubber tires and for preventing various types of rubber goods from adhering to their containers. Such papers must be resistant to mineral oils, edible oils, aromatic oils, butter, lubricating greases, etc. For some of these uses the color or brightness of these papers is of secondary consequence provided that they are sufficiently oil- and greaseproof. But in the case of papers used for the wrapping of foodstuffs or in the making of cartons for this purpose, color is, of course, of great importance.

It has long been known that it is possible to increase the grease resistance of paper and paper boards by coating them with silicate solutions.

2

In the prior art papers and paper boards have also been coated or impregnated with silicate solutions primarily in order to increase their stiffness or crushing strength; also for the purpose of decreasing the penetration and spread of secondary coatings, which are usually much more expensive than silicate coatings. These methods, however, have been seriously limited in their applications, due to the fact that almost all paper stocks, especially the cheaper grades, contain components which are subject to alkali staining, that is components which produce an objectional yellow or brown discoloration when contacted with the alkali present in silicate solutions. It is possible to avoid this staining by the use of purified pulps or pulps consisting substantially of cellulosic components. But the high cost of these pulps makes this method prohibitive for most industrial applications. Prior to the present invention no low-cost method was known of producing papers and paper boards resistant to oils and greases or of increased stiffness and/or of decreased permeability from low-grade paper stocks without impairment of their brightness. The present invention is, of course, not limited to low-grade papers but is applicable in the case of all papers containing materials which are discolored by alkaline solutions.

The paper pulps which are most widely used for the making of papers and paper boards of the type described above are (1) the so-called mechanical or ground-wood pulps prepared by grinding the wood stock without chemical treatment, (2) the semi-chemical pulps produced by a combination of chemical and mechanical steps, (3) the chemical pulps—sulfite, sulfate and soda—in which the original wood chips are thoroughly cooked to a pulp in chemical solutions and which, for this purpose, are not today usually fully bleached even though used for high-grade stocks and (4) re-worked mixtures of the aforesaid pulps. The first of the above classes of pulps contains substantially all of the original non-cellulose constituents of the wood from which it is produced, including lignin and tannin components which turn dark when treated with alkali, while all classes contain at least some components subject to alkali staining, which components can be removed only by thoroughgoing purifying operations. It is evident therefore that papers made from these pulps usually cannot be coated by any treatment in which they are contacted with alkaline solutions without producing deterioration in their color. In addition some papers which are to be coated have

already been coated or sized with materials such as starch or resins which may be discolored by alkaline solutions and therefore cannot usually be coated without producing deterioration in the color of the sheet.

I have discovered that papers of the above type can be coated with alkali metal silicate solutions and their color improved over like products of the prior art if small amounts of bleaching agents are added to the silicate solutions, sufficient in amount to counteract part or all of the staining tendency of the alkali present in the silicate solutions and, if desired, sufficient to improve the color or brightness of the paper. In order to produce this result certain critical conditions must be employed and precautions observed. Thus, I have found that the silicate solutions must have viscosities such that penetration of the paper is only partial, that is, viscosities advantageously within the range of from about 1.0 to 50 centipoises at 20° C. The silicates employed must have ratios of alkali metal oxide to  $\text{SiO}_2$  within the range of 1:1.6 to 1:4. The silicate solutions should contain from about 8 to 40 per cent silicate solids and should have gravities within the range of about 10° to 33.5 Bé. for an alkali-silicate ratio of 1:4 and about 17° to 55° Bé. for a ratio of 1:1.6. Within the range of silicate ratios which are satisfactory, the more alkaline silicates have higher total solids at the same viscosities. The solutions should be applied with a spread of from about 2 to 30 pounds per 1000 square feet of surface. These spreads will usually leave a dry weight of silicate of soda of about 0.3 to 10 pounds per 1000 square feet of surface, depending on the structure and hydration of the sheet. They should contain sufficient oxidizing agent to produce a bleaching action substantially equivalent to that produced by from about 0.25 to 5.0 per cent by weight of hydrogen peroxide. The solutions may be stabilized if desired with a small amount of a soluble magnesium salt and/or a soluble pyrophosphate.

The above described coating solutions can be applied to the paper at any point after the web is formed and the bulk of the water removed therefrom. If desired, the coating solutions can be applied to the web by means of one or more of the final water boxes of the paper machine. This can be accomplished, for example, by allowing the solution to flow into a water box on the calender stack. The web is run through this solution, the excess solution being squeezed off. The paper then passes through the first set of calender rolls to another water box where it receives another treatment with the coating solution and the paper then passes through the rest of the calender stack. The bleaching action takes place while the paper machine is running at full speed, such as 500 feet per minute, for example. The silicate solids collect in the outer layers of the paper and are dried in place by passage through the rest of the calendar.

It is also possible to apply the silicate solution as the web passes through the so-called size press. At such a stage higher viscosity coating solutions are required. The paper at this point may contain as much as 90 per cent of water.

Somewhat better results are obtained if my coating solutions are applied in a separate operation to the paper. A somewhat more concentrated solution of silicate can be used if this is done. The sheet of paper may be passed through a tank of this solution and then through squeeze

rolls which remove the excess. Or the solution can be applied to the paper by means of conventional transfer rolls followed by removal of the excess. If any excess is left, the coating will be too heavy and it is likely to become brittle and crack. The coating operation is preferably conducted at ordinary temperatures but higher temperatures can be used if necessary. The coated sheet can be given a secondary coating, if desired, either with more silicate or with some other material, or it may be rewound directly into a roll.

In lieu of the above methods, it is possible, of course, to employ any of the usual methods of applying coatings to sheet materials, such as dipping, spraying, brushing operations or by the use of knife or roll spreaders or the like. The gravities and viscosities of the solutions to be used must be governed to some extent by the method of application employed. For example when applied in a separate operation the viscosities of my coating solutions should fall within the upper part of the range of 1.0 to 50 centipoises whereas, if the solutions are applied by means of the water boxes of a paper machine, viscosities within the lower part of this range usually produce best results. And allowance must be made for the moisture content of the paper, the degree of sizing, the type of sizing, etc. If the viscosity is too high, the penetration will be poor, if it is too low, the paper becomes so wet that it is difficult to handle. The viscosity which is satisfactory on a dense hard finished paper is considerably lower than that which will give proper penetration into a porous soft board to produce stiffening thereof. No hard and fast rules can be given which will fit all cases but it is believed that the description given herein will be adequate to enable those skilled in this art to obtain satisfactory results with my process.

The papers and paper boards produced in the manner described are highly resistant to oil and grease, as well as to waxes, lacquers, etc., which may be used as outer coating materials in combination with my silicate coating procedure. They are also resistant to water and are considerably stiffer than the uncoated sheets or boards. They materially reduce the loss of aromatic oils from products wrapped therein and absorption and/or penetration of oils and greases is substantially prevented. If a flexible paper is desired, this can be produced by the use of silicate solutions having ratios of alkali metal oxide to  $\text{SiO}_2$  approaching 1:2 and/or by the incorporation of glycerine or other plasticizing agents in the coating solutions.

If a paper is desired which is substantially water-proof as well as oil and grease resistant, this can be accomplished by coating my papers with an outer coating of paraffin or other water-proofing material after they have been treated by the process described above. My silicate coating process is particularly advantageous when used as a pretreatment in connection with other coating procedures for the reason that the silicate coating definitely limits the penetration and softening of the paper by other coatings, such as paraffin, other waxes and lacquers, for example. This means that a substantial saving is effected in the amount of auxiliary coating material required to produce a continuous film.

My present process should not be confused with conventional bleaching procedures which are employed to bleach paper pulp. It is true, of course, that in the conventional bleaching

process, wherein paper pulp is bleached in bulk, a small amount of silicate, usually up to 8 percent, based on the weight of the pulp may be added to inhibit corrosion, to increase the penetration and to stabilize the bleaching agent. But this silicate is washed out in subsequent operations and no silicate coating remains to stiffen the paper or render it oil and grease proof. The residual bleach liquors are dark brown or even black. It is also true that the quantity of bleaching agent required for a given weight of paper fiber is much greater in the usual bleaching process, presumably because in my process the web is bleached only on its surface and the bleaching solution is more concentrated owing to less water being present. Thus, in the bulk bleaching process the pulp is bleached while in suspension in water, only from about 3 to 10 per cent of pulp being present, whereas in contrast, my silicate coatings are applied to the web when the latter usually contains no more than 20 per cent of water. This difference in procedure produces certain surprising results.

For example, if it should be attempted to bleach pulp in the conventional manner employing the proportions of oxidizing agent to pulp which are used in the present process, little or no improvement in color would be obtained and, in the case of sodium hypochlorite, for example, the brightness of the paper would actually be reduced. In addition it is necessary in the bulk bleaching process promptly to remove all residues of the bleaching reaction in order to obviate a substantial reversion in color whereas, in contrast, in my new process the residues are left in the paper and, surprisingly, the reversion in color is small even over a period of several months, much smaller than that which would be produced by the omission of the washing step in the bulk bleaching process. Another surprising fact is that the bleaching action is accomplished in the present process within a period of one or two seconds at a maximum whereas in the bulk process bleaching may require up to several hours.

It should be noted that in my process the bleaching solution usually penetrates the sheet only partially, starting from the outside. The bleaching agent which contacts the outer fibers has a maximum strength while any that penetrates beneath the surface fibers is partly spent. The inner fibers of the sheet therefore cannot be bleached to the same degree as the surface fibers even though they may be partly coated with the silicate. In other words there is a definite gradation in the bleaching of the fibers from the surface to the interior. Since the surface fibers alone are visible this is no disadvantage, and, of course, the saving in bleaching agent which this makes possible is highly important.

An important advantage of my new process is that use can be made of equipment already present in the paper mill or equipment which can be acquired at reasonable cost. On the other hand, a plant for the bulk bleaching of ground wood pulp requires an investment of at least about \$100,000 for a capacity of 50 tons per day. In addition, as pointed out above, in my new process the consumption of bleaching agent is substantially less.

Any of the oxidizing agents can be used in my process which are useful in the bulk bleaching of paper pulp containing ligneous and other materials subject to alkali staining. These oxidizing agents are those which are capable of

dissolving and acting in alkaline solution to release nascent chlorine or oxygen, thereby bleaching these ligneous and other materials. This includes the alkali metal peroxides and hydrogen peroxides; the whole series of colorless soluble per salts, such as the perborates, persulfates, percarbonates, persilicates and the perhalogenates; the soluble hypochlorites; salts of the acidic metal oxides of high valence, such as the halogenates, nitrates, arsenates, antimonates and the like; the polythionates and the products of solution of gaseous oxidizing agents, such as  $\text{Cl}_2\text{O}$ ,  $\text{ClO}_2$  and  $\text{NO}_3$  in alkaline solution. Of course, the same products formed by other means, such as the formation of  $\text{NaOCl}$  by the precipitation of  $\text{Ca}(\text{OH})_2$  from bleaching powder by the addition of caustic, are included. Of these compounds, those equivalent to the nitrates, chlorates, nitrous acid and oxygen itself in alkaline solution are ineffective unless used in high concentration and are therefore less desirable. Those compounds which release nascent oxygen tend to be more effective than those which produce nascent chlorine.

My invention can be described more specifically by reference to the following examples which represent practical embodiments of my coating process applied to the production of my oil- and greaseproof paper.

#### Example 1

3.3 parts of a 30%  $\text{H}_2\text{O}_2$  solution were mixed with 17.7 parts of water and 80 parts of a commercial sodium silicate, known as "S" brand, containing approximately 6.3%  $\text{Na}_2\text{O}$  and 24.6%  $\text{SiO}_2$  (weight ratio of  $\text{Na}_2\text{O} : \text{SiO}_2$  of 1:3.9). This mixture had a gravity of about 27° Bé. and a viscosity of about 9.0 centipoises at 20° C. and an  $\text{H}_2\text{O}_2$  content of about 1%. This solution was surprisingly stable and it was found that 0.6%  $\text{H}_2\text{O}_2$  was still present after standing 24 hours. A sheet of paper made from groundwood pulp was dipped into this solution. A like sheet was dipped into a similar solution to which no peroxide had been added. Another sheet was dipped in water. The sheets were passed through squeeze rolls to remove excess liquid and the sheets were then dried. The sheet which was dipped in water only had a cream-gray color. That dipped into the diluted "S" brand silicate was a dark brown. That dipped into the "S" brand silicate solution containing 1%  $\text{H}_2\text{O}_2$  was light yellow. Samples of these sheets were tested on an Ives Tint-photometer.

The scale of this standard instrument reads from 0-100 and is so adjusted that each of the filters (red, green, blue) reads 100 when tested with a white fresh surface of  $\text{MgO}$ . The readings indicate the parts of red, green and blue light reflected by the sample. A weighted average indicating "brightness" is obtained by summing 70% of green, 20% of blue and 10% of red. The following values were obtained:

|                                              | Red | Green | Blue | Brightness |
|----------------------------------------------|-----|-------|------|------------|
| Water                                        | 64  | 58    | 48   | 57         |
| "S" Brand (80% soin.)                        | 35  | 22    | 27   | 22         |
| 80% "S" Brand with 1% $\text{H}_2\text{O}_2$ | 70  | 61    | 51   | 60         |
| Untreated Sheet                              | 66  | 55    | 49   | 55         |

It is evident that treatment with water had little or no effect but that the presence of 1%  $\text{H}_2\text{O}_2$  increased the whiteness somewhat over that of the original sheet while the sheet treated with

silicate alone was very dark. In 2.5 months the "brightness" of the silicate coated sheet had decreased only 3 points.

#### Example 2

In this test "N" brand sodium silicate was used. This contains approximately 8.9% Na<sub>2</sub>O and 28.7% SiO<sub>2</sub> (weight ratio 1:3.22). The four following coating solutions were prepared:

|                                                                 | 1    | 2    | 3    | 4    |
|-----------------------------------------------------------------|------|------|------|------|
| Parts of 30% H <sub>2</sub> O <sub>2</sub> soln.                | 3.3  | 3.3  | 16.5 | 16.5 |
| Parts of water                                                  | 37.7 | 17.7 | 28.5 | 8.5  |
| Percent H <sub>2</sub> O <sub>2</sub> (approx.)                 | 1    | 1    | 5    | 5    |
| Parts of "N"                                                    | 60.0 | 80.0 | 60.0 | 80.0 |
| Degrees Baumé                                                   | 25   | 34   | 25   | 34   |
| Viscosity (approx.) cp. (at 20° C.)                             | 4.0  | 20.0 | 4.0  | 20.0 |
| Stability, percent H <sub>2</sub> O <sub>2</sub> after 24 hours | 0.4  | 0.3  | 3.2  | 2.2  |

Test samples of the same groundwood pulp paper as used in Example 1 were dipped into these coating solutions, the excess being removed by squeeze rolls as before. The coated samples were then dried and tested on the Ives Tint-photometer with the following results:

|                  | 1      | 2      | 3     | 4     | Original    |
|------------------|--------|--------|-------|-------|-------------|
| Visual color     | Yellow | Yellow | Cream | Cream | Cream-gray. |
| Tint-photometer: |        |        |       |       |             |
| Red              | 71     | 75     | 89    | 94    | 66          |
| Green            | 64     | 65     | 77    | 83    | 55          |
| Blue             | 57     | 52     | 66    | 75    | 49          |
| Brightness       | 63     | 63     | 76    | 83    | 55          |

Although the "N" brand used in this example is more alkaline and therefore would normally cause more discoloration than the "S" brand used in Example 1 it is evident that with 1% H<sub>2</sub>O<sub>2</sub> added it gives a greater improvement than the "S" brand while with 5% H<sub>2</sub>O<sub>2</sub> it gives a very white sheet. After a lapse of 2.5 months tests indicated that the change in brightness of the above samples was within the experimental error.

#### Example 3

Another series of wood pulp paper sheets were coated with solutions of sodium silicates containing various types of bleaching agents and the resulting products tested as before with the Ives Tint-photometer, with the following results:

| Coating Solution                                                                         | Red | Green | Blue | Brightness |
|------------------------------------------------------------------------------------------|-----|-------|------|------------|
| 1. Distilled water                                                                       | 55  | 50    | 41   | 40         |
| 2. 20 p. water and 80 p. "N" brand (blank)                                               | 30  | 20    | 14   | 20         |
| 3. 1.94 p. NaIO <sub>3</sub> , 20 p. water, 80 p. "N"                                    | 35  | 24    | 17   | 24         |
| 4. 3.45 p. NaBO <sub>3</sub> , 2H <sub>2</sub> O, 20 p. H <sub>2</sub> O 80 p. "N" brand | 49  | 34    | 20   | 33         |
| 5. 1.33 p. NaClO <sub>2</sub> , 20 p. water 80 p. "N" brand                              | 45  | 28    | 18   | 28         |
| 6. Cl <sub>2</sub> bubbled into 20 p. water and 80 p. "N" brand                          | 36  | 24    | 19   | 24         |
| 7. ClO <sub>2</sub> bubbled into 20 p. water 80 p. "N" brand                             | 36  | 23    | 14   | 23         |
| 8. 40 p. H <sub>2</sub> O, 60 p. "N" brand (blank)                                       | 43  | 28    | 19   | 28         |
| 9. 41 p. "4.7% NaOCl Soln." 60 p. "N" brand                                              | 50  | 35    | 20   | 34         |
| 10. 5 p. NaClO <sub>2</sub> , 40 p. H <sub>2</sub> O 60 p. "N" brand                     | 71  | 52    | 34   | 50         |

It is evident that all of the above coating solutions, which contain an added oxidizing bleaching agent, produced some improvement in the color of the treated paper sheets in comparison with test sheets treated with corresponding silicate solutions containing no oxidizing agent. Random concentrations were used in the above

tests and my experience has shown that increased brightness can be obtained either by increasing the dilution of the silicate or by increasing the amount of oxidizing agent present. These tests indicate the definite superiority of hydrogen peroxide as an oxidizing agent.

#### Example 4

In this example my process is used in connection with a paper machine producing a 10 point paper containing ground-wood pulp. A coating solution is prepared by diluting 4 parts of "N" brand silicate solution with 1 part of water and adding 2 per cent of hydrogen peroxide. This solution is placed in the pan of a separate coating machine which receives the paper delivered from the paper machine, coats it with the said solution, presses it to remove the excess, leaving a spread of about 10 pounds solution to 1000 square feet of surface, dries it and then winds it on a roll. The so-coated paper has a brightness slightly greater than that of the uncoated paper. The color is substantially stable over a period of several months. The paper is satisfactorily oil- and greaseproof. The consumption of silicate and hydrogen peroxide in this coating process amounts to about 26.6 pounds of the "N" brand silicate and 0.7 pound of H<sub>2</sub>O<sub>2</sub> for each 100 pounds of dry pulp. It is therefore evident that the process is relatively inexpensive.

#### Example 5

In this example a coating solution is prepared by mixing 1 part of "N" brand silicate solution with 1 part of water and adding 5 per cent of hydrogen peroxide. This solution, having a gravity of about 21.8° Bé, is fed into two water boxes on the calender stack of a paper machine producing a 16 point paper from a mechanical pulp. The paper web is run through these water boxes and the excess silicate is squeezed off. After passing through the first water box and the first set of calender rolls it passes through the second water box where it receives another coating of the same silicate solution. The paper then passes through the rest of the calender stack. The total application is about 2 pounds of solution per thousand square feet of surface. The bleaching of the surface fibers is very rapid and takes place while the paper machine is operating at full speed, namely 350 feet per minute. The silicate solids, amounting to about 0.4 pound per 1000 square feet of surface, are concentrated in the outer fibers of the paper and dried in place by the action of the calender rolls. The resulting sheet is oil and grease resistant and has a color which is almost white.

#### Example 6

An illustration of the manner in which silicate coatings can be used to impart stiffness to papers and paper boards and to reduce the spread of a subsequently applied water-proof coating is to be found in the art of making paper milk bottles. The paper used in making these bottles should have a high compression strength and it is highly desirable that this paper be non-porous in order to reduce the quantity of the water-proof coating required. Both of these desirable properties can be obtained by coating the paper with a silicate solution. The color or brightness of the paper used is, of course, important and the present invention can be effectively utilized in such manner that the bright-

ness of the paper is either improved or at least maintained at its original value.

In one specific embodiment of this invention as applied to the stock used in making milk bottles, a good grade of manila board, consisting of sulfite and some bleached sulfate pulp is dipped into a solution of "S" brand silicate of soda solution (ratio 1 Na<sub>2</sub>O:3.9 SiO<sub>2</sub>) diluted to 29° Bé. and having a viscosity of about 15 centipoises to which is added 1 per cent of H<sub>2</sub>O<sub>2</sub>. After dipping, the board is passed through a pair of rolls to remove excess silicate and then dried at room temperature. Part of the board treated in this fashion is coated with a polyvinyl type plastic to make it water proof while another part is coated with paraffin in the usual manner.

Milk bottles made from a silicate-impregnated, paraffin-coated stock have a dry crushing strength of at least 10 per cent greater than those made from the same stock without the silicate impregnation. But a silicate-impregnated, polyvinyl-coated stock produces milk bottles having a wet crushing strength averaging about 100 per cent greater than a stock coated with paraffin alone. The brightness of the stock impregnated with silicate is equal to or slightly higher than that of the original uncoated stock, due to the presence of H<sub>2</sub>O<sub>2</sub> in the coating solution. The quantity of polyvinyl resin required to water-proof silicate-impregnated stock in the manner described is so low—due to the decrease in penetration caused by the silicate—that the method described is practical. The reception, by the trade of milk bottles water-proofed in this manner, is excellent.

#### Example 7

An illustration of a silicate coating procedure used to produce a paper board of increased stiffness and water resistance is in the making of memorandum pads from which pencil notations can be removed merely by wiping with a damp cloth. In this application it is essential, of course, that the pad have a good white color.

In a specific embodiment of making such pads, a stiff 26 point combination paper board or Bristol board with a substantially white sulfite facing sheet and a manila back is impregnated or coated with a "B" brand silicate of soda solution diluted to 13.5° Bé. and about 2 centipoise viscosity to which is added sodium peroxide in an amount corresponding to 0.5 per cent H<sub>2</sub>O<sub>2</sub>. The excess solution is removed by passing the board through squeeze rolls. The original whiteness of the facing sheet is retained and the stiffness of the stock is increased by 10 per cent by the impregnation.

Somewhat thinner paper boards are used in the manufacture of filing separators or filing cabinet partitions. If the stock used in making these articles is impregnated with silicate in the same manner, the stiffness is increased by about 20 per cent without detrimental effect on the color.

The coating procedures described above can be varied in such manner that the spread of solution obtained is within the range of about 2 to 30 pounds of solution per 1000 square feet of surface. And the process can be applied to combined paper board and to paper in sheet form, as well as to papers made from semi-chemical pulps or raw or partially bleached chemical pulps. Likewise paper sheets such as the fibrous sheets made from such impure cellulose raw materials as bagasse, pineapple, ramie, esparto, straw fibers, etc., may be coated within the purview of this invention.

5 Cotton, even though it may be unbleached, is usually so nearly pure cellulose, that it is not seriously discolored by the action of alkalies. During the process the materials which ordinarily would be discolored by the alkaline solutions are destroyed or converted into materials which do not discolor. The use of very small amounts of hydrogen peroxide is sufficient to maintain the color of the uncoated sheet while the brightness of the sheet can be improved by the use of coating solutions containing somewhat larger amounts of oxidizing agent ranging up to about 5 per cent by weight.

15 If it is necessary to operate my coating process at temperatures above room temperature, for example when the water boxes of a paper machine are employed to apply the coating solution, it is desirable to add a stabilizing agent thereto. Any of the stabilizing agents, which are useful in producing stabilization of silicate bleaching baths, can be employed in my coating solutions. The most satisfactory of these agents are magnesium silicate, magnesium sulfate and sodium pyrophosphate, alone or in admixture. 20 25 Any water soluble magnesium and pyrophosphate salts are suitable.

30 In the case of one coating solution containing 3.3 parts of a 30 per cent hydrogen peroxide solution, 17.7 parts of water and 80 parts of "N" sodium silicate solution, I found that the addition of 0.8 part of Na<sub>4</sub>P<sub>2</sub>O<sub>7</sub>·10H<sub>2</sub>O and 0.2 part of MgSO<sub>4</sub>·7H<sub>2</sub>O stabilized the solution to such an extent that its oxidizing power at the end of four days was substantially as great as that of a similar solution free from the stabilizing agents after standing 24 hours. This shows what a surprising stabilizing effect is produced by these agents.

35 It is also true that my coating solutions are substantially more stable when made from purified sodium silicate solutions. Thus, use may be made of the so-called "E" brand silicate, a clarified grade having the same ratio of Na<sub>2</sub>O : SiO<sub>2</sub> as "N" brand. In one test I found, for example, 40 that a coating solution made from this silicate, after dilution to 20° Bé. and viscosity of 2.5 centipoises, and originally containing 5.2 per cent H<sub>2</sub>O<sub>2</sub>, retained 4.2 per cent of H<sub>2</sub>O<sub>2</sub> after 24 hours and 1.5 per cent after 4 days. In another test 45 "Star" brand silicate was used. This contains approximately 10.5 per cent of Na<sub>2</sub>O and 26.3 per cent SiO<sub>2</sub>, with a weight ratio of Na<sub>2</sub>O to SiO<sub>2</sub> of 1:2.5. When 5.6 per cent of H<sub>2</sub>O<sub>2</sub> was added to this silicate, 3.2 per cent was retained after 24 hours even though the silicate was used undiluted at 42° Bé.

50 While I have described what I consider to be the best embodiments of my process and product, it is possible, of course, to vary the procedures 55 which have been described to a considerable extent without departing from the purview of this invention. Thus, as mentioned previously, use may be made of any of the usual methods of applying coating solutions to a paper web. 60 Various additions can be made to silicate coating solutions, such as flaked mica and talc, which decrease the permeability of the coated sheets or boards. It is only necessary in order to obtain the benefits of my process to apply the coating 65 solution at some point after the web is formed and after the bulk of the water is removed therefrom. One or both sides may be coated. It is obvious, of course, that my coating solution should not be washed away once it is applied. By this 70 method it is possible for the first time to silicate- 75

coat a paper sheet containing lignous and other materials, normally subject to staining by silicate solutions, with the use of a single coating solution of an alkali metal silicate and a bleaching agent capable of releasing nascent oxygen or chlorine, to produce a sheet which is not only brighter or less discolored than sheets coated with the said silicate solution alone but which may actually be improved in brightness, and without the necessity of washing out the products of the bleaching reaction. It is believed that this is the first time this result has been accomplished.

What I claim is:

1. In the manufacture of greaseproof paper from low-cost paper stocks containing lignin and tannin components subject to staining by alkali, the process which comprises applying to a web of such a paper stock while it is in the process of being made on a paper making machine, from a box mounted on said paper making machine and at a point where said web contains no more than about 20% of water by weight, a sodium silicate solution, having a viscosity within the range of from about 1 to 50 centipoises, sufficiently low to cause the solution to penetrate the web, to increase its stiffness, to decrease its porosity and to render it oil and grease resistant; said silicate solution having a gravity between about 10° and 55° Bé., containing a weight ratio of Na<sub>2</sub>O to SiO<sub>2</sub> within the range of from about 1:1.6 to 1:4 and containing from about 0.25 to 5% of hydrogen peroxide and as a stabilizing agent a mixture of a water soluble pyrophosphate and a water soluble magnesium salt, whereby the brightness of the coated surface of the web is at least as high as that of a web made from the same paper stock without application of said silicate solution; the silicate solution being applied so that no excess is left on the surface and with a spread ranging from about 2 to 30 pounds per 1000 square feet of web surface; and drying the so-applied coating without removing the coating or washing out the residues of the bleaching reaction.

2. In the manufacture of greaseproof paper

from low-cost paper stocks containing lignin and tannin components subject to staining by alkali, the process which comprises applying to a web of such a paper, which web contains no more than about 20% water by weight, a sodium silicate solution, having a viscosity within the range of from about 1 to 50 centipoises sufficiently low to cause the solution to penetrate the web, to increase its stiffness, to decrease its porosity and to render it oil and grease resistant; said silicate solution having a gravity between about 10° and 55° Bé., containing a weight ratio of Na<sub>2</sub>O to SiO<sub>2</sub> within the range of from about 1:1.6 to 1:4 and containing a colorless oxidizing-bleaching agent of the type which bleaches by liberating a nascent gas, selected from the class consisting of chlorine and oxygen, in amount equivalent, with respect to bleachability, to about 0.25 to 5.0% of hydrogen peroxide, whereby the brightness of the coated surface of the web is at least as high as that of a web made from the same paper stock without application of said silicate solution; the silicate solution being applied so that no excess is left on the surface and with a spread ranging from about 2 to 30 pounds per 1000 square feet of web surface; and drying the so-applied coating without removing the coating or washing out the residues of the bleaching reaction.

WILLIAM STERICKER.

References Cited in the file of this patent

UNITED STATES PATENTS

| Number       | Name      | Date          |
|--------------|-----------|---------------|
| 944,957      | Eberhard  | Dec. 28, 1909 |
| 35 2,069,486 | Tilden    | Feb. 2, 1937  |
| 2,107,297    | Kauffmann | Feb. 8, 1938  |
| 2,185,632    | Hill      | Jan. 2, 1940  |
| 2,187,016    | Craig     | Jan. 16, 1940 |
| 40 2,399,981 | Britt     | May 7, 1946   |

FOREIGN PATENTS

| Number  | Country | Date    |
|---------|---------|---------|
| 659,155 | France  | of 1929 |